

# United States Patent [19]

Kawashima et al.

[11]

4,197,122

[45]

Apr. 8, 1980

[54] **PROCESS FOR PREPARING RAW  
PARTICLES OF CADMIUM SULFIDE FOR  
ELECTROPHOTOGRAPHY**

[75] Inventors: **Hirokuni Kawashima, Tokyo;  
Kiyoshi Suzuki, Kawasaki, both of  
Japan**

[73] Assignee: **Canon Kabushiki Kaisha, Tokyo,  
Japan**

[21] Appl. No.: **792,459**

[22] Filed: **Apr. 29, 1977**

[51] Int. Cl.<sup>2</sup> ..... **G03G 5/08; G03G 5/087**

[52] U.S. Cl. ..... **430/94; 423/561 B;  
423/566; 252/62.6; 430/95**

[58] **Field of Search** ..... **96/1.5; 252/501;  
423/561 B, 566**

[56] **References Cited**

**U.S. PATENT DOCUMENTS**

**2,916,678 12/1959 Bube et al. ..... 252/501  
3,647,430 3/1972 Hanada et al. ..... 96/1.5**

**3,743,609 7/1973 Hirata et al. ..... 252/501  
3,754,985 8/1973 Marlor et al. ..... 252/501**

**FOREIGN PATENT DOCUMENTS**

**632340 12/1961 Canada ..... 423/561 B**

**OTHER PUBLICATIONS**

**Sato, "Diffraction Crystallography of Precipitant Cadmium Sulfide" Applied Physics-Japan, vol. 35, No. 6 (1966), pp. 388-392.**

**Primary Examiner—Roland E. Mattin, Jr.**

**Attorney, Agent, or Firm—Fitzpatrick, Cella, Harper & Scinto**

[57] **ABSTRACT**

A process for preparing raw particles of cadmium sulfide for electrophotography comprises reacting a solution containing cadmium ion and hydrochloric acid with hydrogen sulfide to make cadmium sulfide particles deposited from the solution.

**8 Claims, 1 Drawing Figure**

FIG. 1



**PROCESS FOR PREPARING RAW PARTICLES OF CADMIUM SULFIDE FOR ELECTROPHOTOGRAPHY**

**BACKGROUND OF THE INVENTION**

**1. Field of the Invention**

The present invention relates to a process for preparing raw particles of cadmium sulfide for electrophotography.

**2. Description of the Prior Art**

A conventional process hitherto used for preparing raw particles of cadmium sulfide is to introduce hydrogen sulfide gas into a solution containing cadmium ion such as a solution of cadmium sulfate so as to deposit cadmium sulfide particles from the solution. The cadmium sulfide particles prepared by such a conventional process are raw particles for use in the preparation of final cadmium sulfide particles as a photoconductive material for electrophotography. To prepare the final cadmium sulfide particles for electrophotography, it is usually necessary to further treat the above-mentioned raw particles. Various treating methods have been known and used for this purpose. According to one typical treating method, an impurity having a sensitizing effect of the type so-called donor and acceptor is added to the raw particles and the mixture is heated to a high temperature ranging from 400° C. to 700° C. This treatment has the effect to diffuse the impurity into the raw particles and activate them so that sensitized cadmium sulfide particles may be formed. The sensitized cadmium sulfide particles thus obtained are used as a photoconductive material for electrophotography.

Another conventional method used for preparing raw particles of cadmium sulfide is to use a solution containing cadmium ion and ion of impurity element. This solution is reacted with hydrogen sulfide to form raw particles of cadmium sulfide that preliminarily contains impurity. Since the raw particles thus prepared have already contained the necessary impurity, it is allowed to obtain the aimed cadmium sulfide particles in which impurity is diffused i.e. the aimed sensitized particles by an after-treatment with heat, without incorporating any impurity at the treatment. Also, the sensitized cadmium sulfide particles can be used as a photoconductive material for electrophotography. The latter mentioned preparing method has the advantage that the heat treatment can be carried out at a relatively low temperature compared with the former since the necessary impurity has already been contained in the raw particles before the heat treatment. Furthermore, according to the latter method, a better efficiency is attainable in dispersing the impurity.

However, it has been found that these conventional processes have, in common, some drawbacks as to the preparation of the raw particles.

One of the important disadvantages is found in the fact that the final photoconductive cadmium sulfide particles for electrophotography do not exhibit the same and constant electric characteristic. As known to those skilled in the art, it is important that all of photoconductive cadmium sulfide particles for electrophotography obtained by treating raw particles prepared under the same preparing condition should exhibit the same and constant electrophotographic characteristic. This is an essential requirement to make the produce marketable. But, it is impossible to produce good product particles enough to satisfy the requirement accord-

ing to the conventional processes as described above. In particular, the first mentioned conventional process can not satisfy it.

As another drawback of the conventional processes, it is pointed out that the final photoconductive cadmium sulfide particles for electrophotography obtained by the heat treatment of the raw particles prepared by the conventional processes are poor in moisture resisting property. They are apt to absorb atmospheric moisture and therefore the electrophotographic characteristic of the cadmium sulfide particles changes very easily in accordance with the change in atmospheric humidity. With such cadmium sulfide particles it is difficult to make a good electrophotographic photosensitive material stable against moisture.

**SUMMARY OF THE INVENTION**

Accordingly it is the principal object of the present invention to provide a novel process for preparing raw particles of cadmium sulfide which allows to solve the problems involved in the known processes as described above.

Another object of the invention is to provide cadmium sulfide particles sensitized to the light having a long wavelength.

In accordance with the present invention, there is provided a process for preparing raw particles of cadmium sulfide for electrophotography which comprises reacting a solution containing cadmium ion and hydrochloric acid with hydrogen sulfide to deposit cadmium sulfide particles from the solution.

Other and further objects, features and advantages of the invention will appear more fully from the following description.

**BRIEF DESCRIPTION OF THE DRAWING**

The single FIGURE is a graph showing the sensitivities of various electrophotographic photosensitive plates wherein the curves F and G are sensitivity curves of the photosensitive plates made by using raw particles of cadmium sulfide prepared according to the present invention whereas the curves F' and G' are obtained from the photosensitive plates made by using raw particles of cadmium sulfide prepared according to the conventional ones.

**DESCRIPTION OF THE PREFERRED EMBODIMENTS**

The aimed objects of the present invention are attained by depositing the particles of cadmium sulfide resulted from the reaction in the presence of hydrochloric acid. Hydrochloric acid used in the process of the invention contributes to the preparation of cadmium sulfide particles having constant and definite electric characteristic as well as excellent moisture resisting property. Furthermore, the presence of the hydrochloric acid enables to produce highly sensitized cadmium sulfide particles compared with the conventional ones.

As a solution containing cadmium ion, an aqueous solution of a water soluble salt of cadmium is generally used. Examples of water soluble cadmium salt include cadmium sulfate, cadmium chloride, cadmium nitrate, cadmium acetate, cadmium bromide, cadmium iodide and the like. When such a water soluble cadmium salt is dissolved in water, cadmium becomes present in the form of ion in the aqueous solution. As an alternative, the solution containing cadmium ion may be prepared

by dissolving metallic cadmium in an acid solution capable of dissolving it.

The preparation of a solution containing cadmium ion and hydrochloric acid may be carried out either by adding hydrochloric acid to a solution containing cadmium ion or by adding cadmium ion to a solution containing hydrochloric acid. The reaction of the solution containing cadmium ion and hydrochloric acid with hydrogen sulfide can be carried out according to various known methods. The most typical method is to introduce gaseous hydrogen sulfide into the solution. Other methods such as adding a solution of hydrogen sulfide to the solution or adding the latter to the former may be employed for carrying out the reaction.

It is believed that the resultant product of the reaction of the solution containing cadmium ion and hydrochloric acid with hydrogen sulfide, i.e. raw particles of cadmium sulfide contain chlorine resulted from the used hydrochloric acid although the amount of the chlorine may be very small.

The raw particles of cadmium sulfide thus prepared are subjected to a heat treatment so as to make the particles usable as a photoconductive material for electrophotography. During the heat treatment, the raw particles are heated together with impurity element which serves as donor or acceptor, or with a suitable compound containing therein such an impurity element. As a result, the impurity element is diffused (doped) into the cadmium sulfide particles so that activated photoconductive material useful for electrophotography is obtained. As such an impurity element, there are two types of element one of which is called a donor impurity element and the other is an acceptor impurity element. The donor impurity element is generally selected from elements of Group IIIa, Group IIIb and Group VIIa of the Periodic Table. Preferably Al, In, Ga, Sc and halogen such as Cl, Br and I are used which have a relatively shallow donor level. Here it should be noted that the impurity Cl mentioned above is one offered by substance other than hydrochloric acid. Preferable examples of the acceptor impurity element include elements of Group I of the Periodic Table such as Cu, Ag, Au and Li.

To add the impurity element to the raw particles of cadmium sulfide prior to the heat treatment, various procedures can be employed. For example, the impurity element itself may be mixed with the raw particles or a water soluble salt containing the impurity element may be mixed with the raw particles. As a water soluble salt suitable for this purpose, mention may be made of sulfate, nitrate and cyanate of the impurity element including the following examples:  $\text{Al}_2(\text{SO}_4)_3$ ,  $\text{In}_2(\text{SO}_4)_3$ ,  $\text{Ga}_2(\text{SO}_4)_3$ ,  $\text{Sc}_2(\text{SO}_4)_3$ ,  $\text{CuCl}$ ,  $\text{CuCl}_2$ ,  $\text{CuSO}_4$ ,  $\text{AgNO}_3$  and  $\text{Au}(\text{CN})_3 \cdot 3\text{H}_2\text{O}$ .

The amount of diffusion of impurity element affects the photoconductivity of cadmium sulfide. In case of the donor impurity element, the amount of diffusion is preferably in the range of  $1 \times 10^{-4} - 1 \times 10^{-2}$  mol per 1 mol of cadmium sulfide, and for the acceptor impurity element the range of  $2 \times 10^{-5} - 5 \times 10^{-3}$  mol is preferable.

The incorporation of impurity element into the cadmium sulfide may be carried out when the raw particles are prepared. In this case, raw particles containing impurity element can be prepared by reacting a solution containing cadmium ion, hydrochloric acid and impurity element with hydrogen sulfide. When the raw particles thus prepared is treated with heat, the aimed cad-

mium sulfide particles in which the impurity element is diffused, is obtained. Before the heat treatment, the impurity element contained in the raw particles is present in a state not yet diffused in the particles.

As impurity element used for preparing a solution containing cadmium ion, hydrochloric acid and impurity element, the impurity element itself or a water soluble salt thereof as mentioned above may be used.

For preparing cadmium sulfide particles in which impurity element is diffused, an additional amount of impurity element may be added to the raw particles that have already contained some amount of impurity element prior to a heat treatment.

The impurity element to be diffused in the cadmium sulfide particles may be either of the two types, donor and acceptor. Since the raw particles of cadmium sulfide according to the invention allow the impurity element to easily diffuse in the particles at the time of heat treatment, the heat treatment may be also carried out without adding any flux.

For the density of hydrochloric acid in the solution containing cadmium ion used in the preparation of raw material, a relatively low density is preferably used. Taking the particle size of raw particles into consideration, a range of from 0.01 N to 0.5 N is recommendable. Speaking of the average particle size, about  $1 - 3\mu$  is a preferable range for it.

Now the invention will be explained more fully by examples and referential examples.

#### EXAMPLE 1

To 2 l of 2 N aqueous sulfuric acid containing 1 mol of cadmium sulfate,  $4 \times 4 \times 10^{-4}$  mol of copper sulfate and  $2 \times 10^{-4}$  mol of indium sulfate, hydrochloric acid was added in such amount that the solution contains 0.02 N hydrochloric acid. After the addition, hydrogen sulfide was introduced to the solution at the rate of 1 l/min. for 60 minutes while keeping the temperature of the solution at 60° C. The resultant cadmium sulfide was washed with water and dried after removing excess of impurity. Then it was heated under a nitrogen atmosphere at 450° C. for 120 minutes. After the heat treatment, it was again washed with water and dried to obtain cadmium sulfide for electrophotography.

To the cadmium sulfide thus prepared, there was added 10% by weight (based on the weight of the cadmium sulfide) of vinyl chloride/vinyl acetate copolymer resin and thoroughly dispersed. Thereafter the resultant mixture was coated onto a support plate of aluminum so as to form a photoconductive layer  $40\mu$  thick on the support and dried. In addition, a polyester film  $25\mu$  thick was overlaid on the photoconductive layer to make a photosensitive plate.

Using the photosensitive plate, an image forming was carried out with a copying machine the basic process of which includes the steps of charging with positive polarity, image-wise exposure with simultaneous discharging and whole surface exposure. An image having a good sharpness and a high resolution was obtained.

Also, an image forming was carried out using the same photosensitive plate, but under the condition of high humidity. A clear image that was hardly affected by moisture was obtained.

To evaluate the moisture resisting property of the photosensitive material, the plate was allowed to stand over night under the moisture of 100% R.H. and then the moisture absorption of the photosensitive layer was

measured according to the Karl Fischer's method. The moisture content in the layer was found to be 2100 ppm.

#### REFERENTIAL EXAMPLE 1

Cadmium sulfide was prepared in the same manner as described in Example 1 with the exception that hydrochloric acid was not added this time. Using the cadmium sulfide, a photosensitive plate was made in the same manner as described in Example 1 and an image was formed on it in accordance with the procedure described in Example 1. An image having a good sharpness was obtained. But when an image forming was carried out under the condition of high humidity, a reduction in image density was observed in the formed image. In the same manner as in Example 1, the moisture absorption of the photosensitive plate was measured. The moisture content was found to be 4800 ppm. This means that the moisture resisting property of this photosensitive plate was not so good.

#### EXAMPLE 2

To 2 l of 2 N aqueous sulfuric acid containing 1 mol of cadmium sulfate,  $10 \times 4^{-4}$  mol of copper sulfate and  $15 \times 10^{-4}$  mol of indium sulfate, hydrochloric acid was added in such amount that the solution contains 0.5 N hydrochloric acid. After the addition, hydrogen sulfide was introduced to the solution at the rate of 1 l/min. for 120 minutes while keeping the temperature of the solution at 40° C. The resultant cadmium sulfide was washed with water and dried after removing excess of impurity. Then it was heated under a nitrogen atmosphere at 450° C. for 120 minutes. After the heat treatment, it was again washed with water and dried to produce cadmium sulfide for electrophotography.

Using the cadmium sulfide thus prepared, a photosensitive plate was made and an image forming was carried out in the same manner as in Example 1. An image having a good sharpness and a high resolution was obtained. Also, when an image forming was carried out under the condition of high humidity, there was produced an image having an excellent sharpness which was hardly affected by moisture. The photosensitive plate was allowed to stand in the moisture of 100% R.H. over night and then the moisture absorption of the photosensitive layer was measured. The moisture content in the layer was found to be 1500 ppm.

#### REFERENTIAL EXAMPLE 2

Cadmium sulfide was prepared in the same manner as described in Example 2 with the exception that hydrochloric acid was not added this time. Using the cadmium sulfide, a photoconductive plate was made in the same manner as described in Example 1 and an image was formed on it according to the procedure described in Example 1. An image having a good sharpness was obtained. But when an image forming was carried out under the condition of high humidity, a reduction in image density was observed in the formed image. In the same manner as in Example 1, the moisture absorption of the photosensitive plate was measured. The moisture content was found to be 4500 ppm. This means that the moisture resisting property of this photosensitive plate was not so good.

#### EXAMPLE 3

To 2 l of 2 N aqueous sulfuric acid containing 1 mol of cadmium sulfate,  $8 \times 4^{-4}$  mol of copper sulfate and  $10 \times 10^{-4}$  mol of indium sulfate, hydrochloric acid was

added in such amount that the solution contains 0.3 N hydrochloric acid. After the addition, hydrogen sulfide was introduced to the solution at the rate of 1 l/min. for 120 minutes while keeping the temperature of the solution at 50° C. The resultant cadmium sulfide was washed with water and dried after removing excess of impurity. Then it was heated under a nitrogen atmosphere at 450° C. for 120 minutes. After the heat treatment, it was again washed with water and dried to produce cadmium sulfide for electrophotography.

Using the cadmium sulfide thus prepared, a photosensitive plate was made and an image forming was carried out in the same manner as in Example 1. An image having a good sharpness and a high resolution was obtained. Also, when an image forming was carried out under the condition of high humidity, there was produced an image having an excellent sharpness which was hardly affected by moisture. The photosensitive plate was allowed to stand in the moisture of 100% R.H. over night and then the moisture absorption of the photosensitive layer was measured. The moisture content in the layer was found to be 1900 ppm.

#### REFERENTIAL EXAMPLE 3

Cadmium sulfide was prepared in the same manner as described in Example 3 with the exception that hydrochloric acid was not added this time. Using the cadmium sulfide, a photosensitive plate was made in the same manner as described in Example 1 and an image was formed on it according to the procedure described in Example 1. An image having a good sharpness was obtained. But when an image forming was carried out under the condition of high humidity, a reduction in image density was observed in the formed image. In the same manner as in Example 1, the moisture absorption of the photosensitive plate was measured. The moisture content was found to be 4500 ppm. This means that the moisture resisting property of this photosensitive plate was not so good.

#### EXAMPLE 4

An aqueous sulfuric acid was prepared so as to contain 1 mol of cadmium sulfate,  $10 \times 10^{-4}$  mol of copper sulfate and  $15 \times 10^{-4}$  mol indium sulfate and to have 0.3 N hydrochloric acid in it. To 2 l of the solution, there was introduced hydrogen sulfide at the rate of 1 l/min. for 60 minutes. The resultant cadmium sulfide was washed with water and dried after removing excess of impurity. Then the product was heated in a nitrogen atmosphere at the temperature of 450° C. for 120 minutes. After the heat treatment, it was again washed with water and dried. Thus cadmium sulfide for electrophotography was prepared.

The above described process for the preparation of cadmium sulfide was repeated five times in the entirely same manner so that five samples of cadmium sulfide were obtained each of which corresponds to each run of the five processes respectively.

To each of the five samples of cadmium sulfide thus prepared, 10% by weight of vinyl chloride/vinyl acetate copolymer resin was added and uniformly dispersed. The resultant mixture was coated onto a support plate of aluminum to form a photoconductive layer 40 $\mu$  thick on the support and dried. Thereafter, a polyester film 25 $\mu$  thick was overlaid on the photoconductive layer to make a photosensitive plate.

In this manner, the following five photosensitive plates A through E were manufactured:

Photosensitive Plate A=photosensitive plate manufactured by using cadmium sulfide prepared by the first run process.

Photosensitive Plate B=photosensitive plate manufactured by using cadmium sulfide prepared by the second run process. 5

Photosensitive Plate C=photosensitive plate manufactured by using cadmium sulfide prepared by the third run process.

Photosensitive Plate D=photosensitive plate manufactured by using cadmium sulfide prepared by the fourth run process. 10

Photosensitive Plate E=photosensitive plate manufactured by using cadmium sulfide prepared by the fifth run process. 15

A voltage was applied to each the photosensitive plates with an electrode and the voltage then applied to the photoconductive layer was measured. When  $\oplus$ 2000 V and  $\ominus$ 2000 V were applied, the voltages measured at the respective photoconductive layer were as follows:

| Photosensitive<br>Plate | Applied Voltage |                  |
|-------------------------|-----------------|------------------|
|                         | $\oplus$ 2000 V | $\ominus$ 2000 V |
| Voltage                 |                 |                  |
| at                      |                 |                  |
| Photocon-               |                 |                  |
| ductive                 |                 |                  |
| layer                   |                 |                  |
| A                       | 320 V           | - 1000 V         |
| B                       | 270 v           | - 980 V          |
| C                       | 300 V           | - 1030 V         |
| D                       | 310 V           | - 1050 V         |
| E                       | 250 V           | - 11 950 V       |

From the above table, it will be understood that cadmium sulfide prepared according to the invention exhibits almost the same and constant characteristic through all the runs and the irregularity in characteristic is very small.

#### REFERENTIAL EXAMPLE 4

Into a 2 N aqueous sulfuric acid containing 1 mol of cadmium sulfate, a gaseous stream of hydrogen sulfide was introduced at the rate of 1 l/min. As the product of the reaction, cadmium sulfide was precipitated. After 45 washing the precipitate with water and drying it, completely,  $10 \times 10^{-4}$  mol of copper sulfate and 2% by weight (based on the weight of cadmium sulfide) of cadmium chloride serving as flux were added and mixed with the cadmium sulfide to form a homogeneous mixture. The mixture was then fired at the temperature of 450° C. After the firing it was again washed with water and dried. Thus cadmium sulfide for electrophotography was prepared.

The above described process for the manufacture of cadmium sulfide was repeated five times in the entirely same manner so that five samples of cadmium sulfide were obtained each of which corresponds to each run of the five processes respectively. 55

Using these samples of cadmium sulfide, the following five photosensitive plates A' through E' were manufactured in the same manner as described in Example 4:

Photosensitive Plate A'=photosensitive plate manufactured by using cadmium sulfide prepared by the first run process.

Photosensitive Plate B'=photosensitive plate manufactured by using cadmium sulfide prepared by the second run process.

Photosensitive Plate C'=photosensitive plate manufactured by using cadmium sulfide prepared by the third run process.

Photosensitive Plate D'=photosensitive plate manufactured by using cadmium sulfide prepared by the fourth run process.

Photosensitive Plate E'=photosensitive plate manufactured by using cadmium sulfide prepared by the fifth run process.

A voltage was applied to each the photosensitive plates with an electrode and the voltage then applied to the photoconductive layer was measured. When  $\oplus$ 2000 V and  $\ominus$ 2000 V were applied, the voltages measured at the respective photoconductive layer were as follows:

| Photosensitive<br>Plate | Applied Voltage |                  |
|-------------------------|-----------------|------------------|
|                         | $\oplus$ 2000 V | $\ominus$ 2000 V |
| Voltage                 | A'              | 400 V            |
| at                      | B'              | - 800 V          |
| Photocon-               | C'              | - 1100 V         |
| ductive                 | D'              | - 900 V          |
| layer                   | E'              | - 8500 V         |

From the above table, it will be understood that cadmium sulfide prepared above has a large irregularity in characteristic each other through the five runs.

#### EXAMPLE 5

In the same manner as that of Example 4, but using this time a 2 N aqueous sulfuric acid so prepared as to contain 1 mol of cadmium sulfate,  $4 \times 10^{-4}$  mol of copper sulfate and  $10 \times 10^{-4}$  mol of indium sulfate, and to have 0.3 N hydrochloric acid contained in it, a photosensitive plate F was manufactured.

Also, in the same manner as in Example 4, a photosensitive plate G was manufactured. But, this time there was used a 2 N aqueous sulfuric acid containing 1 mol of cadmium sulfate,  $6 \times 10^{-4}$  mol of copper sulfate and  $12 \times 10^{-4}$  mol of indium sulfate and having 0.5 N hydrochloric acid contained therein.

These photosensitive plates F and G were passed to the process of electrophotography as described in Example 1 to evaluate the sensitivity of the plates. From the measurement of sensitivity, the curve F of FIG. 1 was obtained from the photosensitive plate F and the curve G from the plate G. These curves show that the photosensitive plates F and G exhibit a good sensitivity also to the light in the range of long wave length.

#### REFERENTIAL EXAMPLE 5

To 1 mol of cadmium sulfide prepared by introducing hydrogen sulfide to cadmium sulfate,  $2 \times 10^{-4}$  mol of copper chloride and 2% by weight (based on the weight of cadmium sulfide) of cadmium chloride were added and thoroughly mixed to form a homogeneous mixture. Then the mixture was fired at 450° C. for 100 minutes. The fired mixture was washed with water and dried. Thus cadmium sulfide for electrophotography was obtained. In the same manner as in Example 4, a photosensitive plate F' was manufactured by using the cadmium sulfide.

Also a photosensitive plate G' was manufactured by using cadmium sulfide which was prepared as follows:

To 1 mol of cadmium sulfide prepared by introducing hydrogen sulfide to cadmium sulfate,  $6 \times 10^{-4}$  mol of copper chloride and 2% by weight (based on the weight

of cadmium sulfide) of cadmium chloride were added and mixed to form a homogeneous mixture. The mixture was fired at 450° C. for 100 minutes. Washed with water and dried, the fired mixture gave the aimed cadmium sulfide.

These photosensitive plates F' and G' were tested to evaluate their sensitivity in the same manner as in Example 5. The sensitivity curves F' and G' shown in FIG. 1 were obtained from the photosensitive plates F' and

charging and whole surface exposure. An image having a good sharpness and a high resolution was obtained.

#### EXAMPLES 7-13

5 The process and procedure of Example 6 were repeated under various different conditions. Data of starting materials, final products and reaction conditions used for these examples are summarized in the table given below.

| Example No. | Starting materials             |                                   |       | HCl density (N) | Reaction conditions |             | Firing conditions |             | Final Product Particle size (μ) |
|-------------|--------------------------------|-----------------------------------|-------|-----------------|---------------------|-------------|-------------------|-------------|---------------------------------|
|             | Donor (× 10 <sup>-4</sup> mol) | Acceptor (× 10 <sup>-4</sup> mol) |       |                 | Temp. (°C.)         | Time (min.) | Temp. (°C.)       | Time (min.) |                                 |
| 7           | In 15                          | Cu 10                             | 0.5   | 25              | 120                 | 450         | 120               | 1.5         |                                 |
| 8           | Ga 10                          | Cu 6                              | 0.1   | 25              | 120                 | 480         | 120               | 1.2         |                                 |
| 9           | In 8                           | Au 6                              | 0.1   | 80              | 60                  | 420         | 120               | 3.0         |                                 |
| 10          | In 6                           | Cu 4                              | 0.005 | 80              | 60                  | 450         | 120               | 2.0         |                                 |
| 11          | In 10                          | Ag 5                              | 0.1   | 60              | 120                 | 500         | 120               | 2.5         |                                 |
| 12          | Al 20                          | Cu 8                              | 0.3   | 40              | 100                 | 450         | 120               | 2.0         |                                 |
| 13          | Sc 10                          | Cu 6                              | 0.1   | 60              | 60                  | 450         | 120               | 2.0         |                                 |

G' respectively.

These curves show that the sensitivities of the photosensitive plates F' and G' are inferior to those of the photosensitive plates F and G according to the invention.

#### EXAMPLE 6

21 of a 2 N aqueous sulfuric acid was prepared which contained  $4 \times 10^{-4}$  mol of Cu and  $4 \times 10^{-4}$  mol of In per 1 mol of cadmium sulfate. As Cu and In, the corresponding sulfates were used. To the solution thus prepared, hydrochloric acid was added in such amount that the solution contained 0.02 N hydrochloric acid therein. After the addition, the temperature of the solution was raised up to 60° C. and hydrogen sulfide was introduced into the solution at the flow rate of 1 l/min. for 60 minutes. The resultant cadmium sulfide from the reaction mixture was washed with water and dried after removing excess of impurity. Then the cadmium sulfide was treated with heat in a nitrogen atmosphere at 450° C. for 120 minutes. After the heat treatment, the product was again washed with water and dried. Thus cadmium sulfide having 2.0μ of particle size was obtained.

The cadmium sulfide was dispersed into a vinylchloride vinylacetate copolymer and the dispersion was coated onto a support plate of aluminum to form a photoconductive layer 40μ thick on the support. After drying the coating, a polyester film 25μ thick was overlaid on the photoconductive layer to make a photosensitive plate.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 94

added and at the room temperature (25° C.) hydrogen sulfide was introduced to the solution at the flow rate of 1 l/min. for 120 minutes. A yellow precipitation of cadmium sulfide was obtained.

After washing the cadmium sulfide with water and making it dry,  $6 \times 10^{-4}$  mol of In and  $4 \times 10^{-4}$  mol of Cu were added to it. Thereafter, the product was fired in a nitrogen atmosphere at the temperature of 450° C. for 120 minutes. Cadmium sulfide having about  $2.0\mu$  of particle size was obtained. Using the cadmium sulfide thus obtained, a photosensitive plate was made according to the procedure as described in Example 6 and an image forming was carried out through the same electrophotographic process as that in Example 6. An image having an excellent sharpness and a high resolution was obtained.

#### EXAMPLES 20-23

According to the process of Example 19 where both of donor impurity and acceptor impurity were added to cadmium sulfide at the time of firing, four samples of cadmium sulfide were prepared as shown in the following table. Also, using these samples of cadmium sulfide, excellent results similar to that of Example 6 were obtained.

sulfide for electrophotography as claimed in claim 2 wherein said impurity element ion is an ion of an element selected from the group consisting of In, Al, Ga, Sc, Cl, Cu, Au and Ag.

5 4. A process for preparing raw particles of cadmium sulfide for electrophotography as claimed in claim 1 wherein said solution is an aqueous sulfuric acid solution of metallic cadmium.

10 5. A process for preparing raw particles of cadmium sulfide for electrophotography as claimed in claim 2 wherein said donor impurity element is an element selected from the group consisting of the elements of Groups IIIa, IIIb and VIIa of the Periodic Table, and wherein said acceptor impurity is an element selected from the group consisting of the elements of Group I of the Periodic Table.

15 6. In a process for preparing raw particles of cadmium sulfide for electrophotography which comprises reacting hydrogen sulfide with cadmium sulfate by 20 passing hydrogen sulfide gas through an aqueous solution of cadmium sulfate to deposit cadmium sulfide particles from the solution, the improvement comprising using as said aqueous solution an aqueous solution comprising said cadmium sulfate in the presence of 25 excess sulfuric acid and added hydrochloric acid in a

| Example No. | HCl density (N) | Reaction conditions |             | Firing conditions             |                                  |             | Final product |                         |
|-------------|-----------------|---------------------|-------------|-------------------------------|----------------------------------|-------------|---------------|-------------------------|
|             |                 | Temp. (°C.)         | Time (min.) | Donor ( $\times 10^{-4}$ mol) | Acceptor ( $\times 10^{-4}$ mol) | Temp. (°C.) | Time (min.)   | particle size ( $\mu$ ) |
| 20          | 0.4             | 35                  | 130         | In 20                         | Cu 8                             | 450         | 90            | 1                       |
| 21          | 0.2             | 65                  | 130         | Al 30                         | Ag 10                            | 450         | 90            | 3                       |
| 22          | 0.06            | 45                  | 130         | Ga 10                         | Ag 6                             | 450         | 90            | 1                       |
| 23          | 0.02            | 75                  | 130         | In 6                          | Cu 6                             | 450         | 90            | 2                       |

What we claim is:

1. A process for preparing raw particles of cadmium sulfide for electrophotography which comprises reacting a solution containing cadmium sulfate and added hydrochloric acid with hydrogen sulfide to deposit cadmium sulfide particles from the solution.

2. A process for preparing raw particles of cadmium sulfide for electrophotography as claimed in claim 1, wherein said solution further contains at least one impurity element ion selected from the group consisting of a donor impurity and an acceptor impurity.

3. A process for preparing raw particles of cadmium

concentration of from 0.01 to 0.5 N.

7. A process for preparing raw particles of cadmium sulfide for electrophotography as claimed in claim 6 wherein said aqueous solution further contains at least 40 one impurity ion selected from the group consisting of a donor impurity and an acceptor impurity.

8. A process for preparing raw particles of cadmium sulfide for electrophotography as claimed in claim 7 wherein said impurity element ion is an ion of an element selected from the group consisting of In, Al, Ga, Sc, Cl, Cu, Au and Ag.

\* \* \* \* \*